

3,507,660

PHOTOGRAPHIC MATERIALS CONTAINING  
LONG-CHAIN ALKYL SUCROSE URETHANE  
Fukihiko Nishio, Masakazu Yoneyama, and Yoshinori  
Tuchiya, Ashigara-Kamigun, Kanagawa, Japan, assignors  
to Fuji Shashin Film Kabushiki Kaisha, Ashigara-  
Kamigun, Kanagawa, Japan

No Drawing, Filed Nov. 26, 1965, Ser. No. 510,090  
Claims priority, application Japan, Nov. 26, 1964,  
39/66,280

Int. Cl. G03c 1/38

U.S. Cl. 96—114.5

7 Claims

## ABSTRACT OF THE DISCLOSURE

A gelatin containing photographic composition and a photographic light-sensitive element are disclosed. The composition contains from .05 to 100 g. per 1 kg. of dry gelatin of one of the following compounds:



wherein R is an alkyl group of from 7 to 16 carbon atoms. The element contains a support and a photographic silver halide emulsion layer and the emulsion contains the above compound.

The present invention relates to photography and, more particularly to a gelatin-containing photographic material mainly composed of gelatin for photographic films or photographic papers, said material containing a long-chain alkyl sucrose ether or urethane. By incorporating such a surface active agent as mentioned above in a photographic gelatin layer, that is, a photographic emulsion layer and/or a protective layer, the wetting property of the layer with the surface of a support can be improved and uniform coating can be formed on the support.

It has been variously reported to add natural or synthetic surface active agents in various photographic coating solutions to improve the properties thereof. However, there is trouble in the case of adding natural surface active agents that the quality of the surface active agent is not always constant. On the other hand, it has been reported that by the addition of conventionally known surface active agents, various advantages can be obtained besides improving the wetting property. That is, an antistatic property is endowed, the photographic processing solution can be easily diffused, the troubles caused by water drops can be reduced, air bubbles formed in the case of applying a gelatin sol on a cold-set emulsion surface can be extinguished, development can be accelerated, and staining of a support by a halation preventing dye can be prevented. However, since almost all of the synthetic surface active agents are very peculiar to these actions, although they are effective for some specific photographic emulsions or gelatin compositions, they are sometimes useless to other compositions for

improving wettability or preventing the formation of repellances. Therefore, most of the synthetic surface active agents can be used only within a restricted range of use. For these reasons, there have been provided uses of many different types of surface active agents for photography.

One of the most difficult problems is uniformly coating colloidal silver suspended in a diluted gelatin solution. In this case, it is considered to be impossible to obtain a uniform suspension of colloidal silver and to coat it on surfaces without the formation of bubbles and repellences.

Therefore, an object of this invention is to provide an improved gelatin-containing solution having improved coating property.

Another object of this invention is to provide a photographic emulsion or a gelatin composition not accompanied by repellences and other coating troubles.

An additional object of this invention is to provide a photographic gelatin layer on which a second gelatin layer can be easily coated by applying both layers on a support through separate coating means or by simultaneously applying them on a substratum cooled in a wet state.

25 A further object of this invention is to provide an antistatic effect in the case of coating a coating solution upon a film support.

A still further object of this invention is to provide a coating process while maintaining a coating solution stable, such that no precipitates are formed even in the case of melting at a high temperature.

These and other objects of this invention will become clear in view of the following descriptions.

The inventors have found that these objects can be achieved by adding in a coating solution a long chain alkyl sucrose ether or urethane.

It is considered that the above long-chain monoalkyl sucrose ether and urethane can be shown by the following general formula:



wherein R represents an alkyl group containing from 7 to 16 carbon atoms. In this case, if the carbon number is less than 7, the compound has no surface-active property and, if the carbon number is higher than 16, the compound becomes insoluble in water. In both cases the objects of this invention become unattainable.

The surface active agent in this invention may be added in a photographic coating solution in an amount of 0.05—100 g. per 1 kg. of dried gelatin, and preferably in an amount of 0.1—50 g.

By the addition of the surface active agent, the surface tension of the coating solution is remarkably lowered, the coating solution becomes free of bubbles, and extremely uniform coating can be obtained not only by usual-speed coating, but also by high-speed coating. Further, if a large amount of the surface active agent is incorporated in a photographic emulsion, it does not give

yellow fogging which is inevitably accompanied with the use of other conventional nonionic surface active agents. It also does not have a bad influence on the photographic properties. Furthermore, the surface active agent of the invention may be used together with other known surface active agents.

#### Example 1

A silver bromochloride photographic emulsion containing 7% gelatin and 5% silver halide was prepared. Into the thus prepared photographic emulsion was added the monododecyl ether or sucrose in an amount of 0.5 g. per 1 kg. of emulsion. The photographic emulsion was coated on a baryta paper and set by cooling without drying. On the thus coated layer there was coated a gelatin solution containing di-2-ethylhexyl sodium sulfosuccinate in an amount of 0.2 g. in 1 l. of the 2.5% gelatin solution and it was dried after setting by cooling. The thus obtained photographic emulsion layer and the protective film layer were satisfactory. That is, no bubbles were observed in either the photographic emulsion layer or the protective film layer, and they could be applied at a high speed as compared with that by usual coating method.

#### Example 2

Coating was conducted in the same manner as in Example 1, but using sucrose monododecyl urethane as the surface active agent. This case gave satisfactory results as in Example 1.

#### Example 3

A silver bromo-chloride photographic emulsion containing 7% gelatin and 5% silver halides was prepared. Into the photographic emulsion was added sucrose monododecyl urethane varying the amount in a range of 0.1-3.2 g. per 1 kg. of photographic emulsion. In this case, the sucrose monododecyl urethane was added as a 2% aqueous solution. The emulsion was coated on a baryta paper and dried. The number of repellences and oil spots on thus obtained emulsion-coated photographic papers were investigated in various concentrations of the surface active agent and the results are shown in the following table, which shows that the numbers of repellences and oil spots are effectively reduced by an increase in the addition amount of the surface active agent.

| Concentration of the surface active agent in emulsion (g./kg.) | Number of repellences (No./10 sq. m.) | Number of oil spots (No./10 sq. m.) |
|----------------------------------------------------------------|---------------------------------------|-------------------------------------|
| 0                                                              | 30                                    | 75                                  |
| 0.1                                                            | 11                                    | 12                                  |
| 0.2                                                            | 8                                     | 10                                  |
| 0.4                                                            | 2                                     | 5                                   |
| 0.8                                                            | 1                                     | 3                                   |
| 1.6                                                            | 0                                     | 1                                   |
| 3.2                                                            | 0                                     | 1                                   |

#### Example 4

The procedure as in Example 3 was repeated using sucrose monododecyl ether, which showed as in Example 3, that the number of repellences and oil spots is remarkably reduced as the amount of the surface active agent is increased.

#### Example 5

A photographic silver chloro-bromide emulsion containing 7% gelatin and 5% silver halides was prepared. Into the thus prepared photographic emulsion were added sucrose mono-dodecyl urethane (S.M.D.U.) and sodium dodecyl sulfate (S.D.S.) as a 1% aqueous solution in various proportions. The thus prepared emulsion was coated on a baryta paper and dried. By the procedures, it was confirmed that the number of formed repellences and oil spots were influenced by the balance of the addition amounts of both surface active agents. The results are shown in the following table.

| S.M.D.U., g./kg. Em. | S.D.S., g./kg. Em. |        |        |        |        |
|----------------------|--------------------|--------|--------|--------|--------|
|                      | 2                  | 4      | 8      | 16     | 32     |
| 0.1                  | 6(8)               | 10(11) | 11(15) | 23(18) | 48(37) |
| 0.2                  | 2(6)               | 3(5)   | 6(4)   | 9(15)  | 25(20) |
| 0.4                  | 0(2)               | 0(2)   | 1(2)   | 0(0)   | 1(6)   |
| 0.8                  | 0(1)               | 0(1)   | 0(0)   | 0(0)   | 2(2)   |
| 1.6                  | 0(1)               | 0(1)   | 1(1)   | 0(1)   | 0(0)   |

In the preceding table, a number in the parenthesis represents the number of oil spots in 10 sq. m. and a number outside the parenthesis represents the number of repellences in 10 sq. m.

From the above results is was found that the surface properties of the coated baryta papers were very improved in the range of the balance of the addition amounts (S.M.D.U.:S.D.S.) being 3:1 to 8:1.

#### Example 6

Into 1 l. of an aqueous solution containing 60 g. of gelatin was added 25 g. of colloidal silver. Into the suspension were added as hardening agent 1 g. of 40% formaline and 2 g. of sucrose monododecyl ether. The dispersion was at 40° C. coated on a tri-acetyl cellulose support in a dry-film thickness of 2.0-2.5 microns. There were no bubbles in the coating composition and the thus coated antihalation layer was not accompanied by the formation of repellences. The properties of surface were very excellent.

#### Example 7

A high-sensitivity photographic emulsion for X-ray photography containing 7% gelatin and 6% silver iodobromide was prepared. Into the photographic emulsion was added sucrose mono-dodecyl urethane in an amount of 0.2 g. per 1 kg. of emulsion. The photographic emulsion was coated on a triacetyl cellulose support and, without drying, was set by cooling. On the thus formed layer there was applied a gelatin solution containing sodium long-chain alkylbenzene sulfonate in an amount of 0.1 g. per 1 l. of a 2.5% gelatin solution and, after setting by cooling, the coating was dried. In this case, no bubbles were observed in both photographic emulsion layer and protective layer. Also, the coatings were applied with a sufficient speed. Moreover, the photographic film obtained by this process has very excellent anti-static properties.

What is claimed is:

1. A gelatin-containing photographic composition containing the compound:



60 wherein R represents an alkyl group having from 7 to 16 carbon atoms.

2. The gelatin-containing photographic composition as claimed in claim 1 wherein said compound is contained in said composition in an amount of from about 0.05 to 100 g. per 1 kg. of dry gelatin.

3. The gelatin-containing photographic composition as claimed in claim 1 wherein said compound is contained in said composition in an amount of from about 0.1 to 50 g. per 1 kg. of dry gelatin.

4. The gelatin-containing photographic composition as claimed in claim 1 wherein said photographic composition is a photographic silver halide gelatin emulsion.

5. The gelatin-containing photographic composition as claimed in claim 1 wherein said photographic composition is a protective coating composition.

6. A photographic light-sensitive element comprising a support and a photographic silver halide emulsion layer containing the compound:



5

10

wherein R represents an alkyl group having from 7 to 16 carbon atoms.

7. A photographic light-sensitive element comprising a support, a photographic silver halide emulsion layer, and a protective layer containing gelatin, at least one of said layers containing the compound:



20

25

V. R. Gaertner: Journal of the American Oil Chemists Society, "Sucrose Ether and Ester-Linked Surfactants," vol. 38, 1961, pp. 410-418.

Chem. Absts., vol. 64, 1966, 17702 f.

Chem. Absts., vol. 60, 1964, 9350 c.

wherein R represents an alkyl group having from 7 to 16 carbon atoms.

#### References Cited

##### UNITED STATES PATENTS

- |           |         |             |       |         |
|-----------|---------|-------------|-------|---------|
| 3,170,915 | 2/1965  | Gaertner    | ----- | 252-351 |
| 3,220,847 | 11/1965 | Knox et al. | ----- | 96-94   |
| 3,300,413 | 1/1967  | Ames        | ----- | 252-351 |
| 3,314,936 | 4/1967  | Ames        | ----- | 252-351 |

##### FOREIGN PATENTS

- |         |        |          |
|---------|--------|----------|
| 642,936 | 7/1964 | Belgium. |
|---------|--------|----------|

##### OTHER REFERENCES

V. R. Gaertner: Journal of the American Oil Chemists Society, "Sucrose Ether and Ester-Linked Surfactants," vol. 38, 1961, pp. 410-418.

Chem. Absts., vol. 64, 1966, 17702 f.

Chem. Absts., vol. 60, 1964, 9350 c.

NORMAN G. TORCHIN, Primary Examiner

MARY F. KELLEY, Assistant Examiner

U.S. CL. X.R.

25 106-125